

## UNITED STATES PATENT OFFICE

1,991,162

## PROCESS FOR IMPROVING COPPER-TITANIUM ALLOYS

Wilhelm Kroll, Luxemburg, Luxemburg, assignor to Metal & Thermit Corporation, Carteret, N. J., a corporation of New Jersey

No Drawing. Application January 23, 1930,  
Serial No. 422,955. In Germany February 28,  
1929

7 Claims. (CL 148—21.2)

It is generally known that by means of an addition of beryllium to copper, alloys can be produced subject to be hardened, after being subjected to a special improving process, the so-called "aging". These alloys are quenched at high temperatures, preferably between 700° and 1000° C., and considerable hardness is obtained by annealing at a lower temperature, between 250° and 450° C. the so-called aging.

10 Besides, other copper alloys are known which can be highly strengthened by means of a similar aging process. Mention can be made of the ternary copper-silicon alloys with additions of chromium, nickel, cobalt, iron, or manganese, in 15 said alloys, the aging being caused by the solubility of the silicides. Further mention can be made of the copper alloys containing aluminum and a metal of the iron group, such as manganese, as well as the ternary copper alloys with magnesium and tin.

15 I have found that titanium which up to now is scarcely used in alloying practice, and for this reason is of comparatively low value, is able to give valuable properties to copper alloys, inasmuch as these alloys like the above-named, can 20 be improved by means of subsequent aging after being quenched from a higher range of temperature.

The effect of titanium on copper has been the 25 subject of much research work which, however, till now was restricted to examining very impure alloys of copper and titanium, and wholly inexact values concerning the mechanical properties and the electrical resistance, were determined. Moreover, in the tests made till now the ageability of 30 copper-titanium alloys and its great influence on the electrical conductivity have been wholly overlooked.

The mechanical properties of very pure copper-titanium alloys are extremely favourable. Thus 35 the hardness of an alloy with 5 per cent of titanium, still possessing good rolling properties, can be increased from 140 to 225 by quenching from 820° C. in water and subsequently aging at 320° C. for three hours.

40 Another copper-titanium alloy containing 2.15 per cent of titanium showed the following mechanical properties:—

45 Quenched at a temperature of 850° C. a tensile strength of 35.9 kg/mm<sup>2</sup>, an elongation of 32.5 per cent, a reduction of area of 60.9 percent. The same alloy quenched from 850° and aged for 24 hours at a temperature of 350° C., showed a 50 tensile strength of 66.8 kg/mm<sup>2</sup>, an elongation

of 31.2 per cent, a reduction of area of 74.9 per cent.

An alloy containing 3.05 per cent of titanium subjected to the same treatment, gave the following results:—

5 Quenched at a temperature of 850° C. a tensile strength of 42.6 kg/mm<sup>2</sup>, an elongation of 32.5 per cent, a reduction of area of 79.8 per cent, a hardness of 80.4. After quenching from 850° and aging for 24 hours at a temperature of 350° C. 10 it possessed a tensile strength of 73.4 kg/mm<sup>2</sup>, an elongation of 30.0 per cent, a reduction of area of 60.5%, and a hardness of 175.

An extremely high strength with sufficient elongation is obtained by cold-stretching after 15 aging. The alloy with 2.15 percent of titanium after aging and cold-stretching to 43 per cent showed the following figures:

Tensile strength 100.7 kg/mm<sup>2</sup>, elongation 6.5 per cent, reduction of area 38.3 per cent. 20

The alloy with 3.05 per cent of titanium after the same cold-stretching gave the following results:—

Tensile strength 113.4 kg/mm<sup>2</sup>, elongation 6 per cent, reduction of area 38.2 per cent. 25

It is obvious that at a cold-stretching of 43 per cent the workability has not reached its maximum. If the elongation of an alloy with 3 per cent of titanium is lowered to 1 per cent, a tensile strength of 130 to 140 kg/mm<sup>2</sup> can be 30 reached. An alloy with 4 per cent of titanium attains after aging and cold-stretching a tensile strength of 150 kg/mm<sup>2</sup> and an elongation of 1 per cent.

The effect of aging on the electrical resistance 35 is extraordinarily great. The alloy with 3.05 per cent titanium contents for instance has after quenching a resistance of 0.406 ohm/m/mm<sup>2</sup>. After aging for 21 hours at 350° C. the resistance decreases to 0.142 ohm/m/mm<sup>2</sup>, i. e. to almost 40 one third of its previous value. Regarding the lowest resistance to be produced by aging, alloys with smaller titanium contents give more favourable results. Thus an alloy with 2.15 per cent of titanium after aging and cold-stretching 45 to 43 per cent had a resistance of 0.089 ohm/m/mm<sup>2</sup>.

The extremely high tensile strength of this alloy in addition allows of an advantageous use 50 of these alloys for telephone wires or conducting wires. The advantage in comparison with other alloys employed for this purpose, lies in the high elongation of copper-titanium alloys. The tin-bronze with 6 per cent of tin, for example, in the cold-stretched condition only has a tensile 55

strength of 100 kg/mm<sup>2</sup> and an elongation of 0.5 per cent, whereas the copper-titanium alloy with 2.15 per cent of titanium has a 13 times higher elongation and the same tensile strength.

5 For this reason copper-titanium alloys, eventually after even higher cold-stretching, are especially suitable in such cases where big distances are to be bridged over with conduction wires and the electrical resistance is not of decisive significance. In such cases, the copper-titanium alloys, owing to their greater resistance to atmospheric influences, should be given the preference over steel which, in addition, has a considerably higher electrical resistance.

10 15 Ternary copper-titanium alloys may also be used instead of the binary alloys which are relatively difficult to manufacture, and in particular alloys containing metals of the iron group or light metals besides titanium may be employed.

20 Of such alloys mention shall be made of:

Alloys with maximum titanium content of 4 per cent and up to 10 per cent of nickel, chromium, manganese, iron, cobalt, and molybdenum;

25 Alloys with maximum titanium content of 4 per cent and up to 5 per cent of silicon, magnesium, aluminum.

30 The properties of these alloys can be derived from those of the binary copper-titanium alloys. The aging remains comparatively the same, the elongation is relatively somewhat smaller, and the resistance somewhat higher. Corresponding to the addition of the third metal, the tensile strength may be increased for 20 kg/mm<sup>2</sup> at a maximum. These alloys are in general employed for construction purposes, for example for pressed rods, tubes, and so on. Owing to the higher resistance alloys with more constituents are less suitable for conducting purposes.

35 40 The most favourable quenching temperature for binary copper-titanium alloys is between 750° and 850° C. Alloys with more constituents, in particular those with metals of the iron-group, require a higher quenching temperature. The limits within which quenching may be effected, are between 650° C. and the melting point. Alloys quenched at higher temperatures are more soft; they age relatively in a greater degree.

45 50 The most preferable aging temperature is about 350° C. with an aging time of 24 hours. If aging takes place at a higher temperature, a shorter time must be chosen. Alloys with several metals, in particular those with the metals of the iron group, require a somewhat higher aging temperature. In general the aging temperature is between 250° and 600° C.

55 Similar aging effects may be obtained with casting alloys, but these require a longer time of heating before quenching.

60 In many cases, it is sufficient to heat the alloys for some time at a high temperature, and after simple cooling in air quite a considerable hardness can be obtained in the subsequent aging process. Quenching, therefore, is by no means absolutely necessary, cooling down from a higher

range of temperature is sufficient to attain considerable hardness in the aging process.

What I claim is:

1. A process for improving copper-titanium alloys including a predominating amount of copper and some titanium which comprises cooling said alloys from temperatures of about 650° to 1000° C. and then aging them at about 250 to 600° C.

10 15 2. A process for improving copper alloys including 1 to 4 per cent titanium which comprises quenching the said alloys at temperatures of about 650 to 1000° C. and then aging at about 250 to 600° C.

3. The process for treating an alloy consisting substantially of copper and titanium, the titanium being present in the alloy in but minor quantity, said process comprising heating said alloy to a temperature between about 650° C. to 1000° C., quickly cooling the alloy, and then reheating it to a temperature between about 250° C. to 600° C.

20 25 4. The process of treating an alloy consisting substantially of copper and titanium, the titanium being present in but minor quantities, said process comprising heating said alloy to a relatively high temperature, quenching the alloy, and then reheating it to a relatively low temperature to age-harden the alloy.

30 35 5. Heat-hardened copper-titanium alloys containing titanium in quantities ranging from a small but detectable amount up to about 5 per cent by weight, the balance being substantially copper; said alloys having the tensile strength, electrical resistance and other properties produced by a heat treatment comprising heating said alloy to temperatures ranging from about 650° to 1000° C., followed by aging at temperatures of from about 250° to 600° C.

40 45 6. Heat-hardened copper-titanium alloys containing titanium in quantities ranging from a small but detectable amount up to about 4 per cent by weight and also containing up to 10 per cent of additional hardening metals selected from a group consisting of nickel, chromium, manganese, iron, cobalt and molybdenum; said alloys having the tensile strength, electrical resistance and other properties produced by a heat treatment comprising heating said alloy to temperatures ranging from about 650° to 1000° C., followed by aging at temperatures of from about 250° to 600° C.

50 55 7. The process of treating an alloy containing titanium in quantities ranging from a small but detectable amount up to about 4 per cent by weight and also containing up to 10 per cent of additional hardening metals selected from a group consisting of nickel, chromium, manganese, iron, cobalt and molybdenum, said process comprising heating said alloy to temperatures ranging from about 650° to 1000° C., followed by aging at temperatures of from about 250° to 600° C.

WILHELM KROLL.